# EUROPEAN PATENT SPECIFICATION

(11) **EP 0 033 998 B1**
(45) Date of publication and mention of the grant of the patent: **03.08.1983**
(21) Application number: 81200161.8
(22) Date of filing: 11.02.1981
(51) Int. Cl.: C22B 60/02

(54) **Process for recovering uranium from wet-process phosphoric acid**
Verfahren zur Gewinnung von Uran aus nassgewonnener Phosphorsäure
Procédé de récupération de l'uranium à partir d'un acide phosphorique obtenu par voie humide

(30) Priority: 11.02.1980 NL 8000832
(43) Date of publication of application: 19.08.1981
(73) Proprietor: STAMICARBON B.V., NL-6167 AC Geleen (NL)
(72) Inventor: Weterings, Cornelis Antonius M., NL-6171 AP Stein (L.) (NL); Janssen, Johannes Anna, NL-6451 ER Schinveld (NL)
(74) Representative: Roeffen, Wilhelmus Johannes Maria

## Description

The invention relates to a process for recovering uranium from wet-process phosphoric acid by liquid-liquid extraction with organic esters of phosphoric acid.

Such a process is known from Ind. and Eng. Chem.49(1957) No. 4, p. 628-638, in which alkyl phosphates and alkyl pyrophosphates are named as extractants, Ind. Eng. Chem. 11 (1972) No. 1, p. 122-128 and 13 (1974) No. 3, p. 286-291, in which mixtures of alkyl phosphates and trialkylphosphine oxides, and mixtures of alkylphenyl phosphates dissolved in an aliphatic hydrocarbon such as kerosene are respectively named.

A disadvantage of this known process is that only part of the uranium present in the phosphoric acid is extracted, so that multi-stage extraction is necessary. In this extraction process part of the extractant is lost with the phosphoric acid solution, which, with the very high price of the extractant, raises the cost price of the process considerably.

The present invention provides a process by which it is possible to extract uranium from wet-process phosphoric acid with a considerably smaller quantity of extractant than in the known process and in which extractant losses are also considerably lower.

According to the invention, this is achieved by adjusting the sulphate content of the phosphoric acid to be extracted to a value of less than 2 wt.%, calculated relative to the quantity by weight of P₂0₅ in the phosphoric acid, by addition of a compound of a bivalent metal that reacts with sulphate ions to form a sulphate insoluble in phosphoric acid separation of the metal sulphate precipitate formed.

The sulphate content of the phosphoric acid to be extracted is preferably adjusted to a value of less than 0.6 wt.%, calculated relative to the quantity by weight of P₂0₅ in the phosphoric acid.

Examples of suitable metallic compounds are oxides, hydroxides and salts such as carbonates, sulphides, nitrates, phosphates and chlorides of calcium, magnesium and barium. Mixtures of such compounds may also be applied.

A calcium and/or barium compound is preferably applied as metallic compound. Carbonates and sulphides are especially suitable calcium and/or barium compounds, because in application thereof the anions do not remain behind in the phosphoric acid.

The quantity of metallic compound to be added is not critical, it should merely be sufficient to react with an amount of sulphate in the phosphoric acid such that the residual sulphate content is reduced to below 2 wt.%, and preferably below 0.6 wt.%, calculated relative to the quantity by weight of PP5. Preferably, a quantity of metallic compound is applied that is at least equivalent to the quantity of sulphate in the phosphoric acid to be extracted. If a metallic compound is applied that also reacts with other components present in the phosphoric acid, the quantity of metallic compound to be added should be of course be adjusted accordingly.

The metal sulphate precipitate formed after the addition of the metallic compound can be separated from the phosphoric acid in various ways, for example by filtration, centrifugation, decantation. The precipitate contains, in addition to the insoluble metal sulphate formed, part of the fluorine compounds and metallic contaminants present in the wet-process phosphoric acid. The quantity of these contaminants in the precipitate is determined by the nature and quantity of the metallic compound applied and the grade of wet-process phosphoric acid applied, among other factors. The precipitate can be further pnxessed in various ways, optionally with recovery of the original metallic compound reactive with sulphate ions.

The process according to the invention can be applied in combination with various organic esters of phosphoric acid e. g. in combination with a mixture of di(2-ethylhexyl) phosphoric acid and trioctylphosphine oxide in kerosene, or with a mixture of mono- and dioctylphenyl phosphoric acids in kerosene. The uranium can be recovered from the extracting agent by a known method, too, for instance by precipitation using ammonium carbonate.

The process according to the invention can in principle be applied to various grades of wet-process phosphoric acid. Because it has, however, been found that the efficiency of uranium extraction decreases with increasing P₂0₅ content of the phosphoric acid, dilute phosphoric acid is preferably used as starting material, for Instance with a P₂0₅ content of 30 wt.% or lower. It has, furthermore, been found that the uranium extraction efficiency is adversely affected by soluble fluorine compounds in the phosphoric acid. By the process according to the invention, part of these fluorine compounds are separated from the phosphoric acid with the metal sulphate precipitate, so that further removal of the fluorine is not usually necessary. it a wet-process phosphoric acid with a high fluorine content is used as starting material, the fluorine content can be lowered by addition of an excess, relative to the sulphate to be removed, of a reactive metallic compound and/or by addition of silicon compounds optionally mixed with alkali compounds. The fluorine content of the phosphoric acid to be extracted is preferably adjusted to a value of less than 0.7 wt.%, calculated relative to the quantity by weight of P₂0₅ in the phosphoric acid.

It has, furthermore, been found that the uranium extraction efficiency can be increased by adjusting the nitrate content of the phosphoric acid to be extracted to a value of 0.5-5 wt.%, calculated to the quantity of P_{z}0₅. This can be achieved by adding to the phosphoric acid to be extracted a small amount of nitric and/or nitrates, e. g. ammoniumnitrate.

The invention is further elucidated with reference to the following examples.

### Example 1

### Test No. 1

Into a beaker, 100 gram wet-process phosphoric acid with a P₂0₅ content of 30 wt.%, an S0₄ content of 1.5 wt.%, a fluorine content around 1.2 wt.% and a uranium content of 120 ppm was introduced. A 1 wt.% solution of a flocculant was then added under stirring in a quantity of 4 ml flocculant/litre phosphoric acid. The clear upper layer was then separated from the precipitate formed, which contained the greater part of the organic contaminants and inert components of the phosphoric acid.

Into the liquid thus separated a quantity of solid BaCO₃ was added under stirring, in a 40 wt.% excess relative to sulphate. In the process a precipitate was practically instantaneously formed that was subsequently filtered off. Solid potassium chlorate was added to the filtrate in a quantity of 100 mg/100 gram H₃P0₄, after which the mixture was stirred for approx. 5 minutes, thus to convert the tetravalent uranium to the hexavalent state. To the resulting liquid, an extracting agent was added in a volume ratio of 1-2 relative to the phosphoric acid, which agent consisted of a solution of 0.5 mole di(2-ethylhexyl) phosphoric acid and 0.125 mole trioctylphosphine oxide in 1 litre kerosene. The resulting mixture was stirred vigorously for 10 minutes at a temperature of 45 °C.

The mixture was then allowed to stand for 0.5 hour, forming a two-layer system, and the aqueous, H₃PO₄-containing lower layer was then drained off.

Using X-ray fluorescence analysis and liquid scintillation counting, the uranium content of both the drained-off H₃P0₄-containing phase and the extracting agent phase was determined. The results are summarized in Table 1.

### Test No. 2

The process of Test No. was repeated, but using an excess of 10 wt.% BaC0₃ relative to sulphate. The analysis results are again summarized in Table 1.

### Test No. 3

The process of Test No. 1 was repeated, but using a deficiency of 30 wt.% BaC0₃ relative to sulphate. The analysis results are again summarized in Table 1.

### Test No. 4

The process of Test No. 1 was repeated without addition of BaC0₃. The analysis results are summarized in Table 1.

### Test No. 5

The process of Test No. was repeated, with the concentration of sulphate in the solution being adjusted to 1.5 wt.% after separation of the precipitate containing sulphate and fluorine. The analysis results are summarized in Table 1.

D here signifies : quantity by wt. uranium in extraction liquor/quantity by wt. uranium in phosphoric acid after extraction.

It can be clearly concluded from the analysis results (see Test 1, 2, 3 rel. to blank test 4) that the S0₄ content of the liquid to be extracted has a very distinct influence on the uranium extraction efficiency, and that the fluorine content (see Test 5 rel. to blank test 4) exerts much less influence.

### Example 2

### Test No. 6

In the same way as in Example 1, uranium was extracted from phosphoric acid. In this case the uranium in the liquid was not, after separation of the barium-sulphate-containing precipitate, oxidized with potassium chlorate, however, but reduced with iron turnings (4 gram Fe/100 gram H₃PO₄), the solution stirred for 15 minutes, and the undissolved iron subsequently removed with a magnet. The analysis results are summarized in Table II.

### Test No. 7

The process of Test No. 6 was repeated, but adding only a 10 % excess of BaC0₃ relative to sulphate. The results are summarized in Table II.

### Test No. 8

The process of Test No. 6 was repeated, but adding a deficiency of BaC0₃, however. The analysis results are summarized in Table II.

From the analysis results it appears that although the extraction efficiency of the extractant is fairly low on a reduced (U⁴⁺⁻containing) H₃PO₄ solution, the removal of sulphate and fluorine causes, in this case too, a considerable increase in uranium extraction efficiency.

### Example 3

### Test No. 9

The process of Test No. 1 was repeated, but without treating the solution with potassium chlorate. The analysis results are summarized in Table III.

### Test No. 10

The process of Test No. was repeated, but without addition of BaC0₃. The analysis results are summarized in Table III.

## Claims

1. Process for recovering uranium from wet-process phosphoric acid by liquid-liquid extraction with organic esters of phosphoric acid, characterized in that the sulphate content of the phosphoric acid to be extracted is adjusted to a value of less than 2 wt.%, calculated relative to the quantity by weight of P₂0₅ in the phosphoric acid, by addition of a compound of a bivalent metal that reacts with sulphate ions to form a sulfate insoluble in phosphoric acid and separation of the metal sulphate precipitate formed.

2. Process according to Claim 1, characterized in that the sulfate content of the phosphoric acid to be extracted is adjusted to a value of less than 0.6 wt.%, calculated relative to the quantity by weight of P₂0₅ in the phosphoric acid.

3. Process according to either of Claims 1 and 2, characterized in that the sulphate content is decreased by addition of a calcium and/or barium compound and separation of the calcium and/or barium sulphate formed.

4. Process according to any of Claims 1-3, characterized in that calcium and/or barium carbonate or sulphide are added to the phosphoric acid to be extracted.

5. Process according to any of Claims 1-4, characterized in that the fluorine content of the phosphoric acid to be extracted is adjusted to a value of less than 0.7 wt.%, calculated relative to the quantity by weight of P₂0₅, by addition of a compound of a bivalent metal in excess relative to the sulphate and/or addition of a silicon compound or mixture of a alkali metal compound and a silicon compound.

6. Process according to any of Claims 1-5, characterized in that the nitrate content of the phosphoric acid to be extracted is adjusted to a value of 0.5-5 wt.%, calculated relative to the quantity of P205.

7. Process according to Claim 6, characterized in that the nitrate content is adjusted by addition of nitric acid and/or nitrates.

## Patentansprüche

1. Verfahren zur Gewinnung von Uran aus Nassphosphorsäure durch Flüssig-Flüssig-Extraktion mit organischen Phosphorsäureestern, dadurch gekennzeichnet, dass der Sulfatgehalt der zu extrahierenden Phosphorsäure auf einen Wert von weniger als 2 Gew.-%, bezogen auf die Gewichtsmenge von P₂0₅ in der Phosphorsäure, eingestellt wird durch Zusatz einer Verbindung eines zweiwertigen Metalls, die mit Sulfationen reagiert unter Bildung eines in Phosphorsäure unlöslichen Sulfats, sowie Abscheidung der gebildeten Metallsulfat-Ausfällung.

2. Verfahren nach Anspruch 1, dadurch gekennzeichnet, dass der Sulfatgehalt der zu extrahierenden Phosphorsäure auf einen Wert von weniger als 0,6 Gew.-%, bezogen auf die Gewichtsmenge von P₂0₅ in der Phosphorsäure, eingestellt wird.

3. Verfahren nach einem der Ansprüche 1 oder 2, dadurch gekennzeichnet, dass der Sufatgehalt durch Zusatz einer Calcium- und/oder Bariumverbindung sowie Abscheidung des gebildeten Calcium-und/oder Bariumsulfats herabgesetzt wird.

4. Verfahren nach einem der Ansprüche 1-3, dadurch gekennzeichnet, dass Calcium- und/oder Bariumcarbonat oder -sulfid der zu extrahierenden Phosphorsäure zugesetzt werden.

5. Verfahren nach einem der Ansprüche 1-4, dadurch gekennzeichnet, dass der Fluorgehalt der zu extrahierenden Phosphorsäure durch Zusatz einer auf das Sulfat bezogen überschüssigen Menge einer Verbindung eines zweiwertigen Metalls und/oder Zusatz einer Siliciumverbindung oder Mischung einer Alkalimetallverbindung und einer Siliciumverbindung auf einen Wert von weniger als 0,7 Gew.-% eingestellt wird, bezogen auf die Gewichtsmenge von P₂O₅.

6. Verfahren nach einem der Ansprüche 1-5, dadurch gekennzeichnet, dass der Nitratgehalt der zu extrahierenden Phosphorsäure auf einen Wert von 0,5-5 Gew.%, bezogen auf die Menge des P₂0₅, eingestellt wird.

7. Verfahren nach Anspruch 6, dadurch gekennzeichnet, dass der Nitratgehalt durch Zusatz von Salpetersäure und/oder Nitraten eingestellt wird.

## Revendications

1. Procédé pour récupérer de l'uranium à partir d'un acide phosphorique obtenu par voie humide par une extraction liquide-liquide avec des esters organiques d'acide phosphorique, caractérisé en ce que la teneur en sulfate de l'acide phosphorique à extraire est ajustée à une valeur inférieure à 2% en poids, calculée par rapport à la quantité pondérale de P₂0₅ dans l'acide phosphorique, par addition d'un composé d'un métal bivalent qui réagit avec les ions sulfates pour former un sulfate insoluble dans l'acide phosphorique, et séparation du précipité de sulfate métallique formé.

2. Procédé selon la revendication 1, caractérisé en ce que la teneur en sulfate de l'acide phosphorique à extraire est ajustée à une valeur inférieure à 0,6 % en poids, calculée par rapport à la quantité pondérale de P₂0₅ dans l'acide phosphorique.

3. Procédé selon l'une des revendications 1 ou 2, caractérisé en ce qu'on diminue la teneur en sulfate par addition d'un composé de calcium et/ou de barium et séparation du sulfate de calcium et/ou de barium formé.

4. Procédé selon l'une quelconque des revendications 1-3, caractérisé en ce qu'on ajoute du carbonate ou du sulfure de calcium et/ou de barium à l'acide phosphorique à extraire.

5. Procédé selon l'une quelconque des revendications 1-4, caractérisé en ce que la teneur en fluor de l'acide phosphorique à extraire est ajustée à une valeur inférieure à 0,7 % en poids, calculée par rapport à la quantité pondérale de P₂O₅, par addition d'un composé d'un métal bivalent en excès par rapport au sulfate et/ou addition d'un composé de silicium ou d'un mélange d'un composé de métal alcalin et d'un composé de silicium.

6. Procédé selon l'une quelconque des revendications 1-5, caractérisé en ce que la teneur en nitrate de l'acide phosphorique à extraire est ajustée à une valeur de 0,5-5 % en poids, calculée par rapport à la quantité de P₂0₅.

7. Procédé selon la revendication 6, caractérisé en ce que la teneur en nitrate est ajustée par addition d'acide nitrique et/ou de nitrates.
